

No. 857,793.

PATENTED JUNE 25, 1907.

F. H. DANIELS, A. F. BACKLIN & H. K. SWINSCOE.  
METHOD OFrecovering SULFATE CRYSTALS.

APPLICATION FILED APR. 2, 1906.

4 SHEETS—SHEET 1.

Fig. 1.



WITNESSES

R. A. Balderson.  
Warren M. Swartz

Fig. 2.



INVENTORS

Fred H. Daniels  
Axel F. Backlin  
Henry K. Swinscoe  
by themselves  
their attorney

No. 857,793.

PATENTED JUNE 25, 1907.

F. H. DANIELS, A. F. BACKLIN & H. K. SWINSCOE.  
METHOD OFrecovering SULFATE CRYSTALS.

APPLICATION FILED APR. 2, 1906.

4 SHEETS—SHEET 2.

Fig. 3.



WITNESSES

R. A. Balderson.  
Warren M. Gwartz

INVENTORS.

Fred H. Daniels  
Arl F. Backlin  
Henry K. Swinscoe  
by Deacons & Rogers  
the attys

No. 857,793.

PATENTED JUNE 25, 1907.

F. H. DANIELS, A. F. BACKLIN & H. K. SWINSCOE.  
METHOD OF RECOVERING SULFATE CRYSTALS.

APPLICATION FILED APR. 2, 1906.

4 SHEETS—SHEET 3.



WITNESSES

R. H. Alderson,  
Warren U. Gwartz

INVENTORS

Fred H. Daniels  
Avel F. Backlin  
Henry K. Swinscoe  
by Charles R. Palmer  
their atty

No. 857,793.

PATENTED JUNE 25, 1907.

F. H. DANIELS, A. F. BACKLIN & H. K. SWINSOCE.  
METHOD OFrecovering SULFATE CRYSTALS.

APPLICATION FILED APR. 2, 1906.

4 SHEETS—SHEET 4.



WITNESSES

R. A. Balderson  
Warren W. Beatty

INVENTORS

Fred H. Daniels  
Axel F. Backlin  
Henry K. Swinscoe  
by Backlin & Swinscoe  
the 2nd day of April  
1906.

# UNITED STATES PATENT OFFICE.

FRED H. DANIELS, AXEL F. BACKLIN, AND HENRY K. SWINSCOE, OF WORCESTER, MASSACHUSETTS, ASSIGNORS TO AMERICAN STEEL AND WIRE COMPANY, OF WORCESTER, MASSACHUSETTS, A CORPORATION OF NEW JERSEY.

## METHOD OF RECOVERING SULFATE CRYSTALS.

No. 857,793.

Specification of Letters Patent.

Patented June 25, 1907.

Application filed April 2, 1906. Serial No. 309,821.

*To all whom it may concern:*

Be it known that we, FRED H. DANIELS, AXEL F. BACKLIN, and HENRY K. SWINSCOE, of Worcester, Massachusetts, have invented 5 a new and useful Method of Recovering Sulfate Crystals, of which the following is a specification, reference being had to the accompanying drawing, in which—

Figure 1 is a plan view showing one form 10 of apparatus for carrying out our invention; Fig. 2 is a vertical section on the line A—A of Fig. 1; Fig. 3 is a side elevation, partly broken away showing the multiple effects; Figs. 4 and 5 are respectively a plan view 15 and an elevation showing a modified arrangement of the tanks and conveyers.

The purpose of our invention is to provide 20 a cheap and efficient process for recovering sulfate of iron from the liquor which results from the pickling of iron or steel wire, rods, plates, sheets, etc., in an acid bath.

The object of the invention is to provide a process by which a valuable commercial 25 product may be obtained from this liquor in large amounts and at small expense.

The invention is also applicable with suitable changes in the materials of the apparatus, to the recovery of sulfate of copper from the liquor resulting from the pickling of 30 copper, rods, etc.

In the practice of our invention, we take the sulfate liquor from the pickling vats and deliver it to suitable storage tanks 2 in which it is neutralized by the addition of waste iron 35 or steel wire or other iron or steel scrap. These tanks are preferably provided with steam-coils 2<sup>a</sup> to heat the solution somewhat in order to prevent premature crystallizing in the tanks.

When the solution becomes neutralized, that is to say, when the free acid has been 40 substantially satisfied by the iron with which it comes in contact, it is removed by suitable pumps into a settling-tank 3 in which the 45 mechanical impurities present in the liquor are settled by gravity, and from this settling-tank the solution is drawn successively into vacuum evaporators 4, 4', 4<sup>a</sup>, known in the art as multiple effects. A suitable number 50 of these effects may be employed. Each one contains tubes preferably made of cop-

per, and the effects are provided with vacuum-producing apparatus.

The dilute neutralized liquor is supplied to the first effect, where it comes in contact 55 with and circulates within or around the copper tubes, which are filled with or are surrounded by a heating medium, and in this effect a part of the water passes off in the form of vapor. The liquor then passes to 60 the second effect, in which it is further evaporated, and in the same manner to the other effect or effects, where it is finally concentrated. The steam for supplying the coils of the first effect may be exhaust steam or live 65 steam supplied from an outside source, and the steam for the heating-coils of the second effect may be obtained by utilizing the vapor generated by the boiling of the liquor in the first effect. In the same manner the vapor 70 from the second effect may be passed to the coils of the third effect, and so on, the vapors from the liquor in the final effect being passed into a suitable condenser equipped with a vacuum pump. From the final effect 75 the concentrated liquor is delivered by a pump 5 either to the preliminary cooler or settling-tank, or directly into a number of crystallizing-tanks which may be located on 80 a lower floor.

If the intermediate cooler is employed, it may consist as shown, of a conical shell or dome 6 of steel or iron, which may be cooled in any suitable manner, as by an air blast beneath it. The liquor in passing over this 85 dome loses a portion of its heat and consequently crystallizes more readily, and is then passed to the crystallizing-tanks through pipes 7-7. The tank shown as a cooler may be used only as a settling-tank, as described, 90 thus avoiding the forming of crystals in the pipes which convey the liquor therefrom to the crystallizing-tanks.

The crystallizing-tanks 8, 8 may be of any desirable form, such as round, rectangular, 95 or square, and across the tops are laid planks or boards 9, from which are suspended a large number of thin iron slabs or plates 10. These plates preferably extend vertically and reach nearly to the bottoms of the tanks. 100 The crystals form on these slabs as well as on the sides of the tanks, and the mother liquor

is then drawn off and returned to the storage tanks, after which the crystals are preferably shoveled by hand from the crystallizing tanks on to suitable conveyers 10 and 11 extending between the rows of tanks.

In Figs. 4 and 5 we show a modified arrangement of the tanks and conveyers in which the conveyers 12 and 13 discharge upon a cross-conveyer 14. This conveyer again delivers the crystals to an inclined conveyer 15, which discharges into a hopper 16 provided with spouts and gates through which the material may be charged into any desired number of centrifugal driers 17. The larger percentage of moisture may be drawn off from the crystals by centrifugal force in these driers, which may be of any desirable and well known type. The dried crystals are dropped from the bottoms of the centrifugal driers upon an inclined conveyer 18, which in turn delivers them to an overhead conveyer 19 arranged so that the crystals can be unloaded into any of a series of bins. From these bins the crystals may be drawn off through spouts to the railroad cars or charged into barrels in the building.

The process above described is simple and efficient. The crystals are obtained cheaply and in large quantities, and contain a minimum of moisture, and the apparatus which we employ enables the operation to be carried on continuously and with little hand labor.

We do not claim herein the apparatus disclosed, as this is reserved for, and forms the subject-matter of our divisional co-pending application No. 329,002, filed August 3rd, 1906, for apparatus for recovering sulfate crystals.

Within the scope of our invention as stated in the claims, many changes may be made in the form and arrangement of the apparatus and in the steps of the process. Some of the steps of the process may be employed without others, or may be employed in other combinations, since what we claim is:

1. A process of obtaining in a continuous manner a crystalline metallic sulfate which consists in at least partially neutralizing an acid solution of a metallic sulfate by adding the same metal as the base of the sulfate, transferring the solution to a separate vessel where the impurities separate and then withdrawing and evaporating the solution in a vacuum to the crystallizing point, then

transferring it to a crystallizing tank; substantially as described.

2. A process of obtaining in a continuous manner a crystalline metallic sulfate which consists in at least partially neutralizing an acid solution of a metallic sulfate by adding the same metal as the base of the sulfate, maintaining such solution at a temperature above the crystallizing point, then evaporating the solution in a vacuum to the crystallizing point, and then transferring it to a crystallizing tank; substantially as described.

3. A process of obtaining in a continuous manner a crystalline metallic sulfate which consists in at least partially neutralizing an acid solution of a metallic sulfate by adding the same metal as the base of the sulfate, transferring the solution to a separate vessel where the impurities separate and then continuously feeding the neutralized solution by gravity and evaporating the solution in a vacuum to the crystallizing point, then transferring it to a crystallizing tank; substantially as described.

4. A process of obtaining in a continuous manner a crystalline metallic sulfate which consists in at least partially neutralizing an acid solution of a metallic sulfate by adding the same metal as the base of the sulfate, continuously withdrawing the treated solution and concentrating it to the crystallizing point in successive steps under vacuum while maintaining a substantially constant current in the solution and then transferring the concentrated solution continuously to crystallizing tanks; substantially as described.

5. A process of obtaining in a continuous manner a crystalline metallic sulfate which consists in at least partially neutralizing an acid solution of a metallic sulfate by adding the same metal as the base of the sulfate, continuously withdrawing and hot concentrating the solution under vacuum, and transferring the concentrated solution to crystallizing tanks in a substantially continuous manner; substantially as described.

In testimony whereof, we have hereunto set our hands.

FRED H. DANIELS.  
AXEL F. BACKLIN.  
HENRY K. SWINSCOE.

Witnesses

WM. A. BACON,  
H. M. LATHAM.